

Jan. 24, 1939.

J. T. RUTHERFORD ET AL

2,144,855

METHOD OF PREPARING COMPOUNDED LUBRICATING OIL

Filed Sept. 14, 1936

3 Sheets-Sheet 1



Inventors  
JOHN T. RUTHERFORD  
HENRY A. FRANCIS

FIG. 1 by

*J. Madam*  
Attorney

Jan. 24, 1939.

J. T. RUTHERFORD ET AL

2,144,855

METHOD OF PREPARING COMPOUNDED LUBRICATING OIL

Filed Sept. 14, 1936

3 Sheets-Sheet 2



Inventors

JOHN T. RUTHERFORD  
HENRY A. FRANCIS

by

*J. Malone*  
Attorney

FIG. 2

Jan. 24, 1939.

J. T. RUTHERFORD ET AL

2,144,855

METHOD OF PREPARING COMPOUNDED LUBRICATING OIL

Filed Sept. 14, 1936

3 Sheets-Sheet 3



FIG. 3

*Inventors*  
JOHN T. RUTHERFORD  
HENRY A. FRANCIS

by

*J. M. Malone*  
Attorney

## UNITED STATES PATENT OFFICE

2,144,855

METHOD OF PREPARING COMPOUNDED  
LUBRICATING OIL

John T. Rutherford and Henry A. Francis, Berkeley, Calif., assignors to Standard Oil Company of California, San Francisco, Calif., a corporation of Delaware

Application September 14, 1936, Serial No. 100,704

14 Claims.

(Cl. 87—9)

This invention relates to methods of preparing compounded mineral oils and more particularly to a method of preparing liquid lubricating oils which have the property of inhibiting or preventing piston ring sticking in internal combustion engines.

As disclosed in the application of George L. Neely, Serial No. 38,791 filed August 31, 1935, addition of certain metal naphthenates in small quantities to lubricating oils inhibits piston ring sticking in internal combustion engines. The metal naphthenates therein disclosed, prepared by conventional methods, give this highly desirable property to the oil.

It has been found, however, that the particular method of compounding the lubricant affects profoundly the properties of the completed oil and its efficiency for lubrication purposes. This is especially true when the metal naphthenate used in the compounded oil is a basic metal naphthenate.

Accordingly, an object of the invention is to provide a process of compounding mineral oils containing an aluminum naphthenate to obtain a liquid lubricant of free-flowing, non-stringing consistency which has a viscosity within the range normally utilized in internal combustion engine crankcase lubricants.

The invention has as an additional object the production of a compounded mineral oil containing a dissolved basic metal naphthenate in quantity sufficient to impart increased viscosity and stringiness to the oil but having viscosity reduced to a consistency such that the compounded oil will flow readily through the lubrication system of an internal combustion engine.

Another object of the invention is to provide a method of compounding lubricating oils containing basic metal naphthenates to obtain a lubricant which gives lower rates of wear on bearings and other engine parts, than do such compounded lubricants prepared by previously described or known processes.

A further object of the invention is to provide a method of compounding crankcase lubricating oils to obtain a lubricant which has properties that insure against scoring, scratching or uneven wear of closely fitting parts such as piston rings and cylinder walls during the process of breaking in a new engine.

A further object of the invention is to provide a method of reducing the increased viscosity produced in the oil by the presence of a metal naphthenate and to obtain a lubricant having a viscosity approximately that of the original uncom-

pounded oil or at least a viscosity not greater than that which can be readily circulated through the lubricating systems of internal combustion engines.

Another object of the invention is to provide a method of preparing a basic aluminum salt of petroleum naphthenic acids.

The accompanying drawings and following description illustrate a preferred embodiment of the invention:

Figure 1 is a flow sheet showing in diagrammatic form the preparation and purification of sodium naphthenate stock solutions suitable for use in the process of compounding the lubricant.

Figure 2 is a diagrammatic flow sheet illustrating a method of preparing compounded lubricating oils having superior lubricating properties and containing basic aluminum naphthenates.

Figure 3 illustrates, in part schematically, a form of apparatus which may be used for reducing the excessive viscosity of the compounded oil and for other compounding steps.

Examination of the flow sheets indicates that the process embodies two major steps comprising, first, the preparation of naphthenic acids and purified sodium naphthenate stock solution which is disclosed merely by way of example, and second, the compounding of lubricating oils containing basic aluminum naphthenates.

The flow sheet of Figure 1 is believed to be self-explanatory. Study of this diagram shows that a selected petroleum oil containing naphthenic acids is treated with an alkali such as caustic soda to neutralize and extract the naphthenic acids. The extracted acids are then freed from the aqueous solution by addition of sulfuric acid. The free naphthenic acids are next dissolved with a solvent and treated with sulfuric acid to remove undesirable constituents such as tars and color bodies and finally neutralized with an alkali to give a purified aqueous stock solution of water soluble alkali naphthenates.

Similarly, the compounding process disclosed schematically in Figure 2 may be briefly described by pointing out that the purified aqueous sodium naphthenate solution is heated and basic aluminum naphthenate is simultaneously formed and dissolved in oil by adding sufficient caustic alkali to maintain the solution slightly alkaline while concurrently adding an aluminum salt and lubricating oil. The basic aluminum naphthenate-oil curd formed by this process is then steamed, washed with hot water, dehydrated, diluted with more lubricating oil, reduced in vis-

cosity by treatment with steam, compounded with stearic acid, brightened, filtered, colored, and finally cooled.

The following specific example will serve to 5 illustrate the preferred mode of practicing the process of this invention.

*Preparation of naphthenic acids and sodium naphthenate stock solution*

10 In order to avoid emulsion difficulties when extracting the naphthenic acids from petroleum distillates by the following specific method, it has been found that the oil treated should have a boiling range of approximately 500-700° F. 15 Likewise, in order to avoid difficulty with emulsification during the purification of the extracted acids by the method herein specifically described, it has been found that the crude naphthenic acids contained in the distillate and extracted therefrom should have an acid number no lower than approximately 160. Also, crude acids having an acid number greater than approximately 190 (which yield purified acids having an acid number greater than 225-230) are generally undesirable as they have been found to give naphthenates which are more corrosive to parts being lubricated. (Acid number is the weight in milligrams of potassium hydroxide required to neutralize 1 gram of acids.)

The selected distillate is heated to a temperature of from 150 to 160° F., for example, and sufficient 4° Baumé caustic soda added to neutralize the acids in the stock. The mixture is blown slowly with air for one-half hour and allowed to settle for two hours. The aqueous sodium naphthenate solution which has then formed and settled out is separated and drawn off into a storage container.

The above crude sodium naphthenate stock 40 solution is next purified as follows:

45 The sodium naphthenate solution is placed in a suitable container, acidified with sulfuric acid while agitating with air. The naphthenic acids are freed by this treatment from chemical combination with the sodium and the free acids separate as an oily layer on the surface of the conversion water. This conversion water is an aqueous sodium sulfate liquor and is drawn off to be discarded. The naphthenic acid layer is retained in the container and five volumes of a light hydrocarbon solvent are added to each volume of the separated acids. This solution of naphthenic acids is then treated with 87.5% sulfuric acid at the rate of 2 lbs. of acid per gallon of crude naphthenic acids, the sulfuric acid being added in four separate equal dumps. Following each step in the acid treatment the sludge formed is withdrawn. After the acid treatment, the naphthenic acid solution is washed with salt water until free from mineral acidity as indicated by methyl orange, and until free from sulfates.

55 The naphthenic acids, still in solution, are next neutralized and extracted from the hydrocarbon solvent by treatment with 4° Baumé caustic soda solution. The amount of caustic required to neutralize the naphthenic acids is determined in each case by hand sample. The hydrocarbon solvent separates during the neutralization process. The aqueous layer comprises a solution of purified sodium naphthenate and is withdrawn from the container. Sufficient caustic or purified naphthenic acids are added, when necessary, to make the sodium naphthenate solution neutral.

The naphthenic acids in this purified sodium

um naphthenate solution have a higher acid number than that of the acids as originally extracted. For example, where the acid number of one batch of acids originally extracted as crude sodium naphthenate was 181 that of the purified stock obtained from this crude solution was 215.

Typical batch quantities illustrating the above purification process are as follows:

|                                                                       |                      |
|-----------------------------------------------------------------------|----------------------|
| Crude sodium naphthenate stock charged,                               | 10                   |
| bbls.                                                                 | 388                  |
| Neutralization acid-lbs. (15% fuming H <sub>2</sub> SO <sub>4</sub> ) | 6,400                |
| Treating acid, lbs. (87.5% H <sub>2</sub> SO <sub>4</sub> )           | 6,840                |
| Water washed until neutral to methyl orange.                          | 15                   |
| 4° Bé. caustic, bbls.                                                 | 228                  |
| Purified sodium naphthenate stock yield,                              | 290                  |
| bbls.                                                                 | 290                  |
| Total alkalinity                                                      | 21.5 gsm. NaOH/liter |
| Free NaOH                                                             | Nil                  |
| Free acid                                                             | Nil                  |
| Sulfates                                                              | Nil                  |
| Naphthenic acids, acid No. (Mgs. KOH/gm.)                             | 203                  |
| Color, A. S. T. M.                                                    | 2½ 25                |

It should be understood that the process of preparing and purifying the sodium naphthenate stock solution may be carried out either continuously or as a batch operation. The batch method has been described for the sake of simplicity.

Although the above described process constitutes one method of preparing and purifying naphthenate solutions, this invention is not limited to such a method. Various alternative processes may be adopted depending upon the nature 35 of the oil being treated, the molecular weight of the naphthenic acids being extracted and other such factors.

*Compounding lubricating oil containing basic aluminum naphthenate*

Preparation of the basic aluminum naphthenate according to the preferred procedure of this invention involves simultaneous precipitation and dissolution of the naphthenate in a lubricating 45 oil.

The ingredients necessary for a typical batch are:

|                                                                                      |        |
|--------------------------------------------------------------------------------------|--------|
| Purified sodium naphthenate solution-gals..                                          | 500    |
| 50° Bé. caustic soda solution-lbs..                                                  | 120 50 |
| Aluminum sulfate solution (16 gals. water, 448 lbs. of aluminum sulfate (iron free)) | 190    |
| Lubricating oil-gals..                                                               | 900    |

The above quantities yield 1000 gals. of oil 55 containing 10% aluminum dinaphthenate.

Purified sodium naphthenate solution is charged to a tank provided with a compressed air supply or other means for agitation. When necessary, the pH of this solution should be 60 adjusted so that it is neutral or only slightly on the alkaline side, by addition of caustic soda or suitable acid such as sulfuric acid, depending upon whether the original stock is acid, neutral, or too strongly basic. This solution is then 65 heated to approximately 180° F., for example, by means of open steam. The batch is now ready for the conversion to aluminum naphthenate and is thoroughly agitated with air or by other suitable means during the entire conversion process 70 which process involves addition of caustic soda, aluminum sulfate and lubricating oil to the aqueous sodium naphthenate.

To convert the sodium naphthenate to a basic aluminum naphthenate, caustic alkali and alu- 75

5 minum sulfate or other water soluble aluminum salt are preferably incorporated in the sodium naphthenate solution in the relative proportion of 1 equivalent weight of hydroxide per 3 equivalent weights of aluminum. Such a rate of addition will maintain the sodium naphthenate solution alkaline throughout the precipitation process and yield a naphthenate which analyzes as 10  $\text{Al(OH)}_2\text{R}_2$  (where R represents a naphthenate radical). Aluminum mono-naphthenate, that is,  $\text{Al(OH)}_2\text{R}$ , also comprises a satisfactory compounding ingredient. When the latter compound is to be prepared the proportions of caustic alkali and aluminum sulfate should be such that 2 equivalent weights of hydroxide are added per 3 equivalent weights of aluminum. Mixtures of 15 these basic naphthenate compounds also may be used whether prepared separately or simultaneously, as for example by incorporating 1½ equivalent weights of hydroxide per 3 equivalents of aluminum.

20 The lubricating oil is added at a rate sufficient to insure formation of a soft curd from which sulfates are easily washed out and which readily 25 dissolves in lubricating oils, subsequently to be added.

25 The conversion process may either be a batch or continuous operation and incorporation of the 30 above three ingredients (caustic alkali, aluminum sulfate and oil) in the sodium naphthenate solution may be effected either continuously and simultaneously or concurrently in a stepwise manner. For example addition of 1490 cc. of 50° 35 caustic soda, 7.9 gallons of aluminum sulfate solution (equivalent to 18.6 lbs. of aluminum sulfate) and 5 gallons of lubricating oil in a stepwise manner and in the order named while continuously agitating with air, comprises a satisfactory method of incorporation. This cycle of additions is 40 repeated approximately 24 times for the above described batch and until the endpoint is reached as shown by the sudden loss of tendency to foam and by no further precipitation of aluminum naphthenate.

45 After precipitation of the basic aluminum naphthenate by the above mentioned method, the naphthenate is next blown with live steam for approximately 30 minutes, the conversion water removed, and the naphthenate-oil curd finally 50 thoroughly washed several times with hot water. The wash water is drawn off after each washing operation. Approximately 100 gallons lubricating oil is then added to the naphthenate-oil curd, which is next dehydrated by heating to 300° F. to 55 free it of contained water. Approximately 700 gallons of lubricating oil are finally added to the concentrated naphthenate oil solution to give a finished basic aluminum naphthenate concentrate containing 90% lubricating oil and 10% naphthenate. This mixture is heated and agitated 60 until a clear, bright solution free from lumps is obtained.

65 The above aluminum dinaphthenate concentrate is a product of a semi-solid rubbery consistency convenient for storage or shipping purposes but requires further dilution with oil and particular compounding treatments to render it useful as a crankcase lubricating oil.

70 Figure 3 illustrates a form of apparatus used in compounding the finished oil and in reducing its excessive viscosity. This apparatus comprises a closed container 1, provided at the top with an inlet charging line 2 controlled by a valve 3. Conduit 4, controlled by valve 5, provides an outlet 75 for draining the container 1. A manhole 6 in the

top of the container also permits solids and other materials to be introduced into the container.

Conduit 7 controlled by valve 8 supplies steam to a closed heating coil drained by conduit 9.

5 A superheated steam inlet 10 controlled by valve 11 is connected to a distributor 14 for treating the contents of the container with open steam. A compressed air inlet pipe 12 controlled by valve 13 is also connected to the distributor 14 and constitutes a means for agitating the container 10 contents in addition to the steam.

15 A suitable means for exhausting the gases, such as steam, in the container 1 comprises an ejector 17 operated by air supplied from conduit 15 controlled by valve 16.

The procedure followed in the concluding steps of the process which utilize the above described apparatus is illustrated by the following specific example.

20 The container 1 is charged through conduit 2 with 8,500 gallons of mineral crankcase lubricating oil, previously refined and blended to meet the usual specifications. This oil is heated to a temperature above 212°, for example to 225° F., by means of the closed coil supplied with steam 25 through pipe 7. As the oil is being heated some water may accumulate in the bottom of the container. This water should be drawn off and discarded when the oil reaches 210° F. or a temperature slightly thereunder. In order to avoid 30 possible boiling over resulting from vaporization of entrained water, the batch should be carefully watched while passing through the temperature range 210–220° F.

35 Open steam is admitted through distributor 14 from supply line 10. The quality of the steam should be such that condensation of moisture in the oil is prevented. Superheated steam at 55°–60° F. and having 200°–300° of superheat has been found satisfactory. The quantity of 40 steam is increased until the oil is agitated violently thereby (a 2 inch valve nearly wide open).

45 The aluminum dinaphthenate concentrate, previously prepared, is now dumped into the oil through the manhole 6 in quantities sufficient to give a final concentration of approximately 1% basic aluminum naphthenate in the oil. Since the concentrate contains approximately 10% aluminum dinaphthenate the proportion added will be about 1 part concentrate to 9 parts oil. 50

55 The above mixture is treated with the open superheated steam until the viscosity is broken. By the term "breaking" the viscosity is meant destroying the stringy consistency imparted to the oil by the aluminum dinaphthenate even when the naphthenate is present in amounts of as little as 1%. The temperature of the body of the oil during this steam treatment should be maintained above 212° F. and preferably below 250° F.

60 A simple operating test for stringiness is made by placing oil on the fingers and separating them to measure the tendency to string out. A convenient laboratory test comprises measurement of viscosity. When the viscosity drops to within 2½ seconds Saybolt of that of the original oil, 65 the viscosity is considered to be completely broken. An increase in viscosity in the order of 5 seconds Saybolt is regarded as not substantial and therefore permissible in the completed oil.

70 The aluminum dinaphthenate content of the completed oil should be preferably approximately 1% by weight although more or less naphthenate (for example, ¾ to 2%) may be used as circumstances demand. The aluminum dinaphthenate content is determined by diluting the compound- 75

ed oil with neutral ethyl ether and titration of the diluted oil with a standardized alcoholic caustic alkali solution.

Stearic acid is added to the oil after or during the viscosity breaking operation. The oil is agitated until the acid is dissolved. Addition of free fatty acids such as stearic acid in amounts as small as  $\frac{1}{4}\%$  has been found to give the oil the property of preventing scoring or scratching of pistons, piston rings and cylinders under highly adverse conditions such as encountered when breaking in a new engine under heavy loads and/or high speeds.

After the stearic acid has completely dissolved, and the viscosity of the oil is broken, the compounded lubricant is cooled to a temperature of approximately 210-220° F. and blown with air to brighten. While at this temperature the oil is also filtered to improve clarity and general appearance. During the filtering operation it has been found desirable to use a filter aid such as fibrous diatomaceous earth.

As a final step in the manufacture of the oil, bloom and/or other coloring agents may be added to meet desired color specifications. The completed oil is then cooled to a temperature of 80° F. or lower.

An alternative method which has been used in preparing dilute solutions of naphthenates in oil (for example, 1% magnesium naphthenate or 1% aluminum dinaphthenate in oil) involves precipitation of the naphthenate directly in the oil by contacting an emulsion of the water-in-oil type comprising aqueous sodium naphthenate dispersed in mineral oil, with an aqueous solution of the precipitating metal salt. This method is entirely satisfactory for the preparation of normal naphthenates and operative to produce basic naphthenates. However, preparation of basic aluminum naphthenates by this method has been found to yield a product which contains somewhat more free naphthenic acids than obtained by the previously discussed method.

The following specific example illustrates the above alternative emulsion method.

Emulsify 10.5 gallons of purified sodium naphthenate stock solution and 1.25 pounds of NaOH as a 50° Bé. solution in 40 gallons of S. A. E. 40 lubricating oil. To this emulsion add slowly with continued agitation at 180-200° F., 8.0 gallons of aqueous  $Al_2(SO_4)_3$  solution (9.4 pounds of  $Al_2(SO_4)_3$  per gallon). Agitation and heating are continued until the precipitated basic aluminum naphthenate is dissolved in the oil. The oil which contains 5% basic aluminum naphthenate, is diluted with 4 volumes of lubricating oil and the aqueous sodium sulfate liquor separated. The 1% solution of naphthenate in oil is next washed with fresh water using open steam agitation while maintaining the oil at approximately 205° F., to remove sulfates.

Upon removal of sulfates by the above washing operation the completed oil has substantially the same viscosity and consistency as the original uncompounded oil. Consequently, the necessity of a viscosity breaking operation is avoided.

The oil so prepared is compounded with stearic acid brightened, filtered and colored as previously described relative to the first method of preparation.

As repeatedly mentioned throughout this specification, the particular method of compounding the basic aluminum naphthenate lubricant is of critical importance in that it affects profoundly, the lubricating efficiency of the compounded oil.

For example, precipitation of the basic aluminum naphthenate from sodium naphthenate solutions by adding a solution of caustic soda and an aluminum salt solution separately and in proper relative proportions, might appear to be unimportant on superficial examination. As a matter of fact this feature is highly important. The caustic soda should be added at a rate sufficient to maintain the naphthenate solution alkaline yet in quantities insufficient to precipitate substantial quantities of the added aluminum salt as aluminum hydroxide. When this procedure is followed a naphthenate of uniform composition is obtained.

On the contrary if the aluminum salt and caustic solution be mixed together prior to incorporation in the sodium naphthenate solution the soluble aluminum salt is converted to the hydroxide and proper combination with the naphthenic acid ions of the sodium naphthenate solution is obtained only with considerable difficulty, if at all. Similarly if all of the caustic soda is added to the sodium naphthenate solution prior to incorporation of the soluble aluminum salt, the first precipitate formed will comprise principally aluminum hydroxide; aluminum mono-naphthenate will next be formed and as the mixture becomes less and less alkaline the naphthenate formed will comprise first the dinaphthenate and finally the normal aluminum naphthenate will predominate. Such a composite mixture is less desirable for lubrication purposes than the uniform naphthenate obtained by the process of this invention because the mixture appears to be less stable as indicated by a higher corrosion rate on certain bearing metals.

Again, if all of the soluble aluminum salt is first added to the sodium naphthenate, subsequent addition of caustic soda tends to form aluminum hydroxide as a precipitate in the oil and this precipitate recombines with naphthenic acids only with considerable difficulty. This latter proposed method also results in removal of a portion of the naphthenic acids from the oil as sodium naphthenate with the resulting problems of waste or of recovery of these extracted ingredients.

The mineral oil is preferably but not necessarily added during the precipitation process simultaneously with the aluminum sulfate and caustic soda to produce a naphthenate curd containing oil which is more easily washed free from sulfates and can be readily incorporated in oil and dehydrated. If the oil is not added during precipitation the basic naphthenate curd has a high melting point and is difficult to wash, completely dehydrate and incorporate in oil. If the oil is added to the aqueous sodium naphthenate prior to precipitation, the first portion of naphthenate precipitated takes up the oil so that the soap formed toward the end of the precipitation is comparatively free from oil and the same difficulties exist in dehydration and dispersing uniformly in an oil solvent.

Mineral oils compounded with 1% basic aluminum naphthenate in the manner in which mineral castor oil stocks have been prepared, will have viscosities in the order of 500 to 600 (Furol) at 100° F., whereas the mineral oil before compounding will have a viscosity of about one-tenth this figure. Two methods of reducing the viscosity of the compounded oil to essentially that of the original oil can be used.

One method consists of heating the oil to a temperature in excess of 300° F., agitating to

dissolve the naphthenate, and maintaining this temperature for a period of from one to four hours until there is no further reduction in viscosity which is, at this point, essentially the same as the original oil. The time required to complete this operation is dependent upon the temperature and upon the volume of oil being treated, etc. At higher temperatures the time is reduced materially and at temperatures of 250° F. or below the rate of viscosity reduction is so slow that it is not commercially practical.

The other method of reducing viscosity, which is the preferred method described in this specification, comprises steaming the oil with open steam while maintaining the oil at a temperature of from 212-250° F. To prevent condensation of moisture, temperatures above 212° F. are desirable, but not absolutely necessary. This procedure for reducing viscosity avoids oxidation effects resulting from prolonged heating at high temperatures. The upper temperature limit is not critical, but should of course be below the boiling point of the oil. Temperatures above 250° F. are not necessary and oils have been satisfactorily reduced in viscosity by steaming at 230° F. for a period of one-half to one hour.

The nature of the chemical mechanism of the action of the steam during this viscosity breaking operation has not been established. Mere observation of physical effects, however, definitely establishes that open steam in direct contact with the compounded oil greatly accelerates the viscosity breaking operation. This phenomenon is regarded as unpredictable, and perhaps may be properly designated a catalytic one. In addition to its accelerating effect on the viscosity breaking operation, the steam serves to agitate the lubricating oil and to provide a protecting atmosphere above the body of lubricant which prevents oxidation of the oil.

It should be apparent from the previous description that the process of this invention, in its broader aspects, is applicable to preparation of basic naphthenate compounds of poly-valent metals other than aluminum, for example, to preparation of basic iron or chromium naphthenates. Likewise, soluble metal salts other than sulfates or mixtures of salts of different metals can be used during the precipitation process. Various equivalent alkali can also be substituted for the caustic soda for controlling alkalinity of the sodium naphthenate solution during the precipitation process. Also, the viscosity breaking feature of the invention in its broader aspects is not limited to naphthenates but includes oil solutions of organic carboxylic acids in general.

Accordingly, it is desired to include within the scope of this invention the various equivalents embraced within the spirit of the invention and the terms of the appended claims.

We claim:

1. A process of breaking the viscosity of an oil containing sufficient metal naphthenate in solution to substantially increase viscosity and stringiness, which comprises heating said oil at a temperature above 212° F., but below the boiling point of the oil and accelerating the viscosity breaking operation by intimately contacting said oil with open steam.

2. The process of claim 1 in which the naphthenate is an aluminum naphthenate.

3. The process of claim 1 in which the naphthenate is a basic aluminum naphthenate.

4. A process of preparing a basic metal salt of

naphthenic acids which comprises mixing an aqueous solution containing a water-soluble polyvalent metal salt and an aqueous solution containing an alkali naphthenate while maintaining the alkalinity of said mixture above pH 7 but below the point at which substantial quantities of the hydroxide of said poly-valent metal are precipitated by concurrent addition of an alkali, whereby a basic metal naphthenate is precipitated.

5. A process as in claim 4 in which said polyvalent metal is aluminum.

6. A process as in claim 4 in which the pH is regulated during precipitation by incorporation of aqueous caustic soda in the proportion of approximately 1 equivalent weight of sodium hydroxide per three equivalent weights of a tri-valent metal.

7. A process as in claim 4 in which the tri-valent metal is aluminum and the pH is regulated during precipitation by incorporation of aqueous caustic soda in proportions to yield a naphthenate selected from the group consisting of aluminum dinaphthenate, aluminum mono-naphthenate and mixtures of aluminum dinaphthenate and mono-naphthenate.

8. A process of preparing a solution of a basic metal naphthenate in oil which comprises commingling an aqueous solution containing a polyvalent metal capable of forming oil-soluble basic naphthenates with an aqueous solution of a water-soluble naphthenate while in intimate contact with sufficient oil to dissolve the precipitated naphthenate, and maintaining the alkalinity of said mixture above pH 7, but below the point at which the hydroxide of said poly-valent metal is formed in substantial quantities by concurrent addition of an alkali, whereby the basic naphthenate of said poly-valent metal is precipitated.

9. A process of preparing a solution of a basic metal naphthenate in a lubricating mineral oil fraction without substantially increasing the viscosity of the oil, which comprises commingling an aqueous solution containing a polyvalent metal ion, an aqueous solution of a water soluble naphthenate, and said mineral oil fraction, and maintaining the alkalinity of said mixture during said commingling operation above pH 7 but below the point at which the hydroxide of said polyvalent metal is formed in substantial quantities by concurrent addition of an alkali hydroxide whereby a basic naphthenate of uniform composition and minimum free acid content is formed and dissolved in said oil in sufficient quantity to materially increase the viscosity thereof, and breaking the increased viscosity of said oil solution to the consistency of the original oil.

10. A process of preparing a solution of a basic metal naphthenate in a lubricating mineral oil fraction without substantially increasing the viscosity of the oil, which comprises forming said basic naphthenate and simultaneously dissolving the same in said mineral oil in proportions sufficient to materially increase the viscosity of the oil, heating said oil solution to a temperature above 212° F. but below the boiling point of the oil and accelerating the viscosity breaking operation by intimately contacting said oil with open steam.

11. A process of preparing a solution of a basic metal naphthenate in a lubricating oil, said solution being characterized by increased stability and low free acid content as measured by reduced corrosivity to bearing metals, which comprises commingling with an aqueous solution of a water-

soluble naphthenate a solution containing a polyvalent metal ion capable of forming oil-soluble basic naphthenates, maintaining the alkalinity of said mixture above pH 7 but below the point at which the hydroxide of said polyvalent metal is formed in substantial quantities by concurrent addition of an alkali hydroxide, dissolving the polyvalent metal naphthenate in a lubricating oil in quantities sufficient to increase the viscosity and stringiness of said oil, and breaking said viscosity by heating at a temperature above 212° F. but below the boiling point of the oil and until the consistency of said oil is reduced to that at which it will readily flow through the lubrication system of internal combustion engines.

12. The process of claim 11 in which the precipitation is carried out in the presence of a lubricating oil to dissolve the precipitate as formed.

13. A process of preparing a liquid lubricating oil capable of inhibiting piston ring sticking in internal combustion engines which comprises commingling a solution containing a polyvalent metal ion capable of forming oil-soluble basic naphthenates with an aqueous solution of a water-soluble naphthenate, maintaining the alkalinity of said mixture above pH 7 but below the point at which the hydroxide of said polyvalent metal is formed in substantial quantities by concurrent addition of an alkali hydroxide, concurrently adding lubricating oil whereby the basic naphthenate of said polyvalent metal is precipitated in the presence of the lubricating oil, dissolving said

basic naphthenate in the oil in quantities sufficient to increase the viscosity and stringiness of the oil, breaking said viscosity and stringiness by heating at a temperature above 212° F. but below the boiling point of the oil and until the consistency of said oil is reduced to that at which it will flow readily through the lubrication system of internal combustion engines, and accelerating the viscosity breaking operation by directly contacting the compounded oil with open steam. 10

14. A process of preparing a liquid lubricant which comprises dissolving in a mineral lubricating oil a basic metal naphthenate comprising the reaction product of a solution containing a polyvalent metal ion capable of forming oil-soluble basic naphthenates, an aqueous solution of a water-soluble naphthenate, and an alkali hydroxide in an amount sufficient to maintain the alkalinity of the reaction mixture above pH 7 but below the point at which the hydroxide of said polyvalent metal is precipitated in substantial quantities, said naphthenate being dissolved in the oil in a quantity sufficient to substantially increase the viscosity thereof, and breaking the increased viscosity by heating the solution at a temperature above 212° F. but below the boiling point of the oil and until the consistency of said oil is reduced to that at which it will flow readily through the lubrication system of internal combustion engines. 20

JOHN T. RUTHERFORD.  
HENRY A. FRANCIS. 30